

## UNITED STATES PATENT OFFICE

2,108,761

## FIRE RESISTANT PULP BOARD

Hubert L. Becher, Trenton, N. J., assignor to  
Homasote Company, a corporation of New  
Jersey

No Drawing. Application March 28, 1936,  
Serial No. 71,535

12 Claims. (Cl. 92—21)

My invention relates to a pulp board which is highly fire-resistant and to the method of making the same.

My invention is of particular advantage in connection with molded pulp board, such as is usually made by running wood pulp, paper pulp or the like into a mold and by means of pressure removing the majority of the water (see, for instance, United States Letters Patent No. 971,936, dated October 4, 1910, and No. 1,272,566 dated July 16, 1918) and subsequently drying out the remainder of the water by the application of heat. After it has been dried, or simultaneously with the drying, the board may, if desired, be subjected to high pressure in order to compact the same thus giving it higher tensile and transverse strength and a higher degree of hardness. The object of my invention is to produce a pulp board whose fibres are coated with aluminum hydrate to such an extent that the board is highly fire-resistant and will smolder as little as possible, if at all, after having been exposed to a flame, which contains a substantial proportion of incombustible substances, and which has a surface sufficiently hard to resist minor injuries.

It is a further object of my invention to apply aluminum hydrate to fibres in such a manner that when such fibres are molded or otherwise formed into the preliminary shape of the finished board there will be as little interference as possible with the drainage of the water from the pulp and no undue warping of the wet board.

Other objects of my invention will be apparent from the following description thereof.

In order to fireproof the pulp fibres in the best manner known to me, I deposit aluminum hydrate thereupon before they are shaped into the form of a board. I deposit such aluminum hydrate preferably in the form of a precipitate from a double decomposition of an aluminum salt and of some other substance which will react with such aluminum salt to form aluminum hydrate, but not such a substance as will react with the aluminum salt to form insoluble crystals. I prefer to use aluminum sulfate and caustic soda or sodium aluminate, obtaining in each case aluminum hydrate and sodium sulfate, the latter in the form of soluble crystals which eventually will go out with the wash water. The aluminum hydrate when obtained as a precipitate from the double decomposition referred to, is in a fine state of subdivision and will therefore more readily coat each of the pulp fibres. I prefer to cause the reaction between the aluminum sulfate and the caustic soda or other reagent to take place in the beater in which, and while, the pulp is being beaten, first adding the aluminum sulfate and, when this has been thoroughly dissolved in the beater, adding a suspension of caustic soda or other suitable reagent, but I may cause such re-

action, and obtain the precipitated aluminum hydrate resulting therefrom, in a separate vessel, in which event the precipitate should be used as soon as possible to prevent agglomeration thereof.

The proportion of aluminum hydrate is preferably such as will result in as complete a coating of the pulp fibres as possible, but not much more than that, so as not to interfere with the proper felting thereof.

To the pulp which is being beaten in the beater, I add, preferably before adding the aluminum hydrate and other reagent, a substantial proportion of fuller's earth, although I may add this while the reaction is taking place or even afterwards. Preferably at the same time at which I add the fuller's earth, I add to the pulp, while it is being beaten, a substantial proportion of exfoliated vermiculite, although I may do this at a later stage. Preferably, after the reaction has taken place and before adding any sizing (if sizing be added) I add a substantial proportion of asbestos fibres sufficiently short, for instance,  $\frac{1}{8}$  inch in average length, so as not to interfere with the subsequent proper felting of the fibres and the pulp. The fibres are known in the trade as asbestos "floats." My reason for adding the asbestos fibres, if I add them at all, after the reaction has been completed, is that I desire to have the aluminum hydrate coat as fully as possible the fibres of the pulp, which must be fireproofed, the asbestos itself, of course, needing no fireproofing; also to have the asbestos fibres protect the coated fibres. I prefer to render the board waterproof as well as fire resistant, and therefore prefer to add to the beaten mixture of the ingredients hereinabove referred to, the usual soap (sizing) and thereafter to precipitate it onto the fibres.

After the materials hereinabove referred to have been thoroughly mixed, the board is shaped in a mold or otherwise and dried, after which it may, if desired, be compacted; or it may be simultaneously dried and compacted, for instance, in a hot press.

My present preferred formula is the following, by weight:

|                        | Per cent |
|------------------------|----------|
| Pulp (dry)             | 26       |
| Aluminum hydrate       | 6        |
| Asbestos               | 7        |
| Fuller's earth         | 26       |
| Exfoliated vermiculite | 35       |

This formula may be varied, not only by leaving out the asbestos but also by changing the proportions of the remaining ingredients. I have obtained good results by using pulp (dry weight) 25 to 30%, aluminum hydrate 6 to 8%, asbestos 7 to 10%, fuller's earth 25 to 30%, and exfoliated vermiculite 30 to 40%.

I have already indicated that the asbestos may

be omitted, although the board is very much improved by its presence. In place of fuller's earth I may use an equivalent material, such as kaolin, or other finely divided clay, or bauxite, but I 5 have not found as yet any equivalent which is as effective as fuller's earth or nearly so as bauxite; care should, however, be taken to use a fuller's earth which is not too dense—for instance, such as I have obtained from England which, I understand, 10 is of the density characteristic of the fuller's earths found in such country, and is not so effective because it is entirely too dense. The main purpose of using this material is not only to avoid using in the fire-resistant board too 15 much of the combustible pulp, but also to assist in hardening the surface of the completed board. The purpose of using exfoliated vermiculite is to obtain very free drainage during the step of removing the water from the pulp, for instance, 20 when the latter is being primarily shaped in a mold, and also to lower the density of the board. Its use is advantageous also because it is completely incombustible.

I prefer to add to the water in the beater, preferably at the end of so much of the process as takes place in the beater, enough calcium chloride, or (as an equivalent) magnesium chloride, or other suitable hygroscopic salt or sodium thiosulfate, to produce a 2% or 3% solution of this 30 material with the water in the beater. The purpose of adding this material is to guard against a deterioration of the aluminum hydrate covering of the individual fibres, if the board should be dried, or exposed to fire, for so long a time as 35 would otherwise cause such deterioration. Of course, such overdrying should be avoided, if possible, but with the addition of either one of these salts the danger of the aluminum hydrate becoming porous or shrinking (because of dehydration) thus exposing some of the fibre, is avoided.

My preferred method (which results in the least costly board) therefore includes the following steps:

45 1. Preparation of a pulp suspension from any suitable fibre, such as wood fibre, chemically digested fibre or mixtures thereof, as can be obtained, for instance, by beating up old newspapers; bagasse or straw may be used in whole or 50 in part. I refer to all such substances in my claims as cellulosic fibres. Enough water should be used to permit the fibres to flow freely.

55 2. Adding to 26 parts by weight of pulp (dry), as it is being beaten in the beater, 26 parts by weight of fuller's earth and 35 parts by weight of exfoliated vermiculite, the beating continuing until all the ingredients have been thoroughly mixed.

60 3. Preparation of aluminum hydrate in the requisite finely divided form, in an amount just about sufficient to coat the fibres, by adding aluminum sulfate to the beater and, when this is dissolved, adding a solution of the requisite amount of sodium aluminate; just about enough 65 of the latter substance should be used to convert the aluminum of the aluminum sulfate into aluminum hydrate; I prefer to use this substance, as the combination of the sodium with the sulfate-ion will also release aluminum hydrate contained in the sodium aluminate. It is advisable that the solution of sodium aluminate be added gradually to the solution of the aluminum sulfate, to give full opportunity to the aluminum hydrate particles to coat fully the pulp fibres. 70 75 The beating should be continued during this step.

Enough aluminum sulfate and sodium aluminate should be added to result in the formation of about 6 parts by weight of aluminum hydrate, keeping in mind that aluminum hydrate is obtained not only from the reaction between the aluminum of the aluminum sulfate, but that the sodium aluminate itself embodies aluminum hydrate. 5

As the pulp is to be subsequently sized, care should be taken to keep or render the mixture 10 in the beater neutral or slightly alkaline, so as to avoid premature precipitation of the soap.

4. Adding to the beater 9 parts of well shredded asbestos fibres, the fibres preferably not exceeding  $\frac{1}{8}$  inch in length, to 26 parts by weight of 15 pulp (dry), the beating being continued until the ingredients are thoroughly mixed.

5. A suitable rosin or other soap, in weight equal to about 2% to 3% of the total weight of the solid materials, is added to the beater charge 20 as a sizing ingredient, preferably after the asbestos, fuller's earth and exfoliated vermiculite have been thoroughly mixed with the pulp.

6. The soap is then precipitated by adding a suitable quantity of a suitable precipitant, such 25 as aluminum sulfate.

7. Calcium chloride (or magnesium chloride) is then added in an amount sufficient to produce a solution of 2% strength with the water in the beater. 30

1-7. Preferably the beating of the pulp, and thereafter of the pulp and other ingredients as the latter are being added, continues throughout the first seven steps so that a thorough mixture 35 of the various ingredients is obtained.

8. The pulp is then shaped in a mold or otherwise, and dried, and compacted. The drying time depends, of course, upon a number of factors, such as the thickness of the board and the amount of water contained therein. Care should 40 be taken not to dry for so long a time as to over dry the board; preferably some moisture is left in it, not only so as to render it less brittle, but also to avoid warping when it is thereafter exposed to the moisture of the atmosphere. 45

The resulting board is sufficiently fire-resistant to comply with the majority, if not all, of the building codes of American cities; incidentally, the product, if waterproofed as above described, is also sufficiently water resistant, to permit its use in construction work exposed to the elements. It has rigidity and good mechanical strength with freedom from brittleness, and a low heat transmission as compared with boards composed principally of mineral products, such as cement, asbestos or plaster. My invention may be employed, with substantially equally good results, in making a pulp board by the laying up process, that is, by forming paper-like layers of the board, for instance, on a paper making machine, and uniting the layers thereof in the usual manner, for instance, with the aid of sodium silicate. 55 60 65

The proportions of material hereinabove given may be varied, as may also the steps and succession of steps outlined in my statement of preferred method, without departing from the spirit of my invention. All of the proportions given hereinabove are approximate. 70

The aluminum hydrate, referred to by me, is  $\text{Al}(\text{OH})_3$ .

I claim:

1. A highly fire resistant substantially hard surface board comprising cellulosic fibres coated with aluminum hydrate and mixed with a sub- 75

stantial proportion of fuller's earth and exfoliated vermiculite.

2. A highly fire resistant substantially hard surface board, as claimed in claim 1, containing, 5 by weight, cellulosic fibres 25 to 30 parts, aluminum hydrate 6 to 8 parts, fuller's earth 25 to 30 parts, and exfoliated vermiculite 30 to 40 parts.

3. A highly fire resistant substantially hard surface board, as claimed in claim 1, comprising, 10 by weight, cellulosic fibres approximately 26 parts, aluminum hydrate approximately 6 parts, fuller's earth approximately 26 parts and exfoliated vermiculite approximately 36 parts.

4. A highly fire resistant substantially hard surface board, as claimed in claim 1, containing also 15 a substantial proportion of asbestos.

5. A highly fire resistant substantially hard surface board as claimed in claim 1, comprising, 20 by weight, cellulosic fibres 25 to 30 parts, aluminum hydrate 6 to 8 parts, fuller's earth 25 to 30 parts, exfoliated vermiculite 30 to 40 parts, and asbestos 7 to 10 parts.

6. A highly fire resistant substantially hard surface board as claimed in claim 1, comprising, 25 by weight, cellulosic fibres approximately 26 parts, aluminum hydrate approximately 6 parts, fuller's earth approximately 26 parts, exfoliated vermiculite approximately 36 parts, and asbestos 7 parts.

30 7. A highly fire resistant substantially hard surface board as claimed in claim 1, containing also from 2% to 3% of a hygroscopic salt suitable to protect the aluminum hydrate from dehydration when exposed to heat.

35 8. A highly fire resistant substantially hard surface board as claimed in claim 1, containing by weight, cellulosic fibres 25 to 30 parts, alumi-

num hydrate 6 to 8 parts, fuller's earth 25 to 30 parts, exfoliated vermiculite 30 to 40 parts and from 2% to 3% of a hygroscopic salt suitable to protect the aluminum hydrate from dehydration when exposed to heat.

5 9. A highly fire resistant substantially hard surface board, as claimed in claim 1, comprising, by weight, cellulosic fibres approximately 26 parts, aluminum hydrate approximately 6 parts, fuller's earth approximately 26 parts, exfoliated 10 vermiculite approximately 36 parts and from 2% to 3% of a hygroscopic salt suitable to protect the aluminum hydrate from dehydration when exposed to heat.

10 10. A highly fire resistant substantially hard surface board, as claimed in claim 1, containing also a substantial proportion of asbestos and from 2% to 3% of a hygroscopic salt suitable to protect the aluminum hydrate from dehydration when exposed to heat.

20 11. A highly fire resistant substantially hard surface board, as claimed in claim 1, containing, by weight, cellulosic fibres 25 to 30 parts, aluminum hydrate 6 to 8 parts, fuller's earth 25 to 30 parts, exfoliated vermiculite 30 to 40 parts, asbestos 7 to 10 parts and from 2% to 3% of a hygroscopic salt suitable to protect the aluminum hydrate from dehydration when exposed to heat.

25 12. A highly fire resistant substantially hard surface board, as claimed in claim 1, containing, by weight, cellulosic fibres 26 parts, aluminum hydrate 6 parts, fuller's earth 26 parts, exfoliated vermiculite 36 parts, asbestos 7 parts and from 2% to 3% of a hygroscopic salt suitable to protect the aluminum hydrate from dehydration 30 when exposed to heat.

35 HUBERT L. BECHER.